

# UNITED STATES PATENT OFFICE.

HUGH RODMAN, OF OAKMONT, PENNSYLVANIA, ASSIGNOR TO RODMAN CHEMICAL COMPANY, OF VERONA, PENNSYLVANIA, A CORPORATION OF PENNSYLVANIA.

## CASE-HARDENING COMPOUND AND METHOD OF MANUFACTURING.

1,372,832.

Specification of Letters Patent. Patented Mar. 29, 1921.

No Drawing.

Application filed June 28, 1920. Serial No. 392,412.

To all whom it may concern:

Be it known that I, HUGH RODMAN, a resident of Oakmont, in the county of Allegheny and State of Pennsylvania, have invented a new and useful Improvement in Case-Hardening Compounds and Methods of Manufacturing, of which the following is a specification.

This invention relates to the art of manufacturing casehardening compounds. It discloses a new material for use in that art and a method of manufacturing a new and improved casehardening compound.

It is old to make a casehardening compound by coking a mixture of a coking substance and an energizing chemical so as to produce large masses of compound coke, which are then broken up and sized to meet commercial requirements. The common practice of this special method consists in mixing ordinary coking coal with soda-ash and lime, all of these ingredients being in dry powdered condition, and then coking this mixture to produce a compound coke containing carbon and the reduced chemicals, this compound coke being subsequently crushed and screened to secure fragments about one-fourth inch in dimension. While a satisfactory casehardening material can be produced by this means, there are several difficulties involved.

One difficulty inherent in the use of coal as the coking agent in the method described above consists in the fact that all coals contain considerable ash, or inert material, which may react with the energizing chemicals, or directly with the steel being carbonized, to produce glassy adhesions upon the surface of the steel, this reaction being particularly noticeable when soda-ash is used as a chemical energizer.

Another difficulty consists in the actual loss of chemical energizer and the consequent reduction of the efficiency of the material, because of the fixing of the chemicals by the ash in chemical combinations which are not effective as energizers. For instance, the soda-ash may combine with the siliceous ash of the coal to produce alkali silicates. These are of little or no use as energizers.

Another difficulty is that the ordinary sulfur content of coking coal, usually above one per cent. of the weight of the coal, may pass to some extent and under conditions which

are not well understood, into the steel, along with the carbon. That is harmful.

Another difficulty consists in the fact that when these large masses of compound coke are crushed there is produced in the crushing operation considerable quantities, generally more than twenty-five per cent. of unmerchantable fine particles and dust, which must be rejected and lost, or else worked up by expensive methods into other products. As explained, coal has been used in this special art, subject to the limitations described. It has also been proposed to mix chemical energizers with crude oil and distill to produce a compound coke for casehardening. While this latter proposal has probably not been commercially put into practice, such a method would undoubtedly have some of the same disadvantages that exist with coal. For example, the product would have a high ash and sulfur content, and the difficulties resulting therefrom would be the same as in the coal compound.

All of these difficulties are overcome by the present invention which consists in the use of the distillates derived from coal as the coking agent in the mixture, instead of the coal itself. Preferably I use the ordinary hard fuel pitch instead of other distillates from coal because there are great quantities of this material produced for which under present conditions little or no market exists, this condition having become accentuated with the recent increase in by-product coke ovens. Such pitch is available in abundance with an ash content of less than one per cent. and a fixed carbon content of fifty-five or sixty per cent. when coked as herein described. This may be compared with the ordinary eight or ten per cent. of ash in coking coal and a fixed carbon content of about sixty-five per cent. in the Pittsburgh coal area.

By mixing the pitch with the energizing chemicals in any convenient manner, and then coking this mixture, I secure a compound coke which has much greater mechanical strength than the similar product made from coal, and of considerably less weight per unit of volume. This latter quality (low specific density) is of value, as the material is used by bulk, rather than by weight. The casehardening efficiency of the pitch base material is also greater than that

2  
of the coal base material, because of the absence of ash in the pitch.

Furthermore the dust and fine fragments produced in crushing the compound coke made from pitch, may be added to the following batch of raw materials going to the coking ovens or stills without reducing the mechanical strength of the coke produced. In other words I am able to re-use the unmerchantable fines and dust by the simple means of recharging them into the still with subsequent raw batches, without loss of mechanical strength in the coke produced; whereas, if the fines and dust from a coal base compound coke are mixed in with subsequent raw batches, a very weak and unsalable casehardening material is produced.

Thus the chief difficulties inherent in the use of coking coal in this special art may be overcome by using the cheap (and generally unmarketable) pitch instead of uncoked coking coal.

Pitch is the hard, brittle product remaining after the lighter oils and chemicals have been removed from ordinary coal tar, and is preferable because of its comparative cheapness and high fixed carbon ratio,—but other distillates of coal, as for example the raw tar, may also be used.

In the practice of my invention any sort of commercial coking apparatus may be used. The chemicals may be mixed with broken up pitch while all the ingredients are solid, then the mixture heated, forming a coked compound, that is then crushed and screened to size. Or, the pitch, or other carbonaceous material may be melted, then the chemicals stirred into the liquid, then the mixture coked, etc. Or the carbonaceous element may be completely coked, crushed and screened, and then the chemicals added and uniformly distributed over the carbonaceous bases, by some such process as described in U. S. Patent 949446. I have made excellent material each way, using about seven parts of soda-ash and twelve parts of lime hydrate with one hundred parts of pitch; and I have mixed the dust and fines resulting from crushing the com-

ound coke so produced with a similar batch 50 of raw materials and produced coke of apparently the same strength as the first batch. Other energizing chemicals may be used. By energizing chemicals I mean such materials as will when added to an inactive carbonaceous substance render such carbonaceous substance active as a carbonizing agent. I have generally coked in bottom fired, metal stills, heating slowly several hours to a temperature of about 1000° Fahr., 60 or at least till the smoke producing distillates have been all given off. The gases may be either used as fuel for the heating furnace, or may be distilled and reused for other purposes. 65

I claim:

1. A casehardening compound comprising coked pitch.
2. A casehardening compound comprising coked pitch, and an energizing chemical. 70
3. A casehardening compound comprising coked mixture of pitch and an energizing chemical.
4. The method of manufacturing a casehardening compound, comprising mixing 75 energizing chemicals with a coal tar base, coking the mixture, crushing and screening to size.
5. The method of manufacturing a casehardening compound, comprising mixing 80 energizing chemicals with pitch, coking the mixture, crushing and screening to size.
6. The method of manufacturing casehardening materials consisting in coking a coal tar base, crushing and screening it to 85 size, and mixing suitable energizing chemicals therewith.
7. The method of manufacturing casehardening materials consisting in coking pitch, crushing and screening it to size, and 90 mixing suitable energizing chemicals therewith.

In testimony whereof I have hereunto set my hand.

HUGH RODMAN.

Witnesses:

JO. BAILY BROWN,  
HOWARD S. SNIVELY.